

D. C. COLLIER.

METHOD OF FORMING ARTICLES OF IMPREGNATED FIBER.

APPLICATION FILED JUNE 21, 1917.

1,372,118.

Patented Mar. 22, 1921.



Inventor:

David C. Collier,

By *Byron Townsend & Brickmire*

Attorneys.

# UNITED STATES PATENT OFFICE.

DAVID C. COLLIER, OF SAN DIEGO, CALIFORNIA, ASSIGNOR TO WILLIAM M. SHEFFIELD,  
OF NEW YORK, N. Y.

## METHOD OF FORMING ARTICLES OF IMPREGNATED FIBER.

1,372,118.

Specification of Letters Patent. Patented Mar. 22, 1921.

Application filed June 21, 1917. Serial No. 176,207.

*To all whom it may concern:*

Be it known that I, DAVID C. COLLIER, a citizen of the United States, residing at San Diego, in the county of San Diego and State 5 of California, have invented certain new and useful Improvements in Methods of Forming Articles of Impregnated Fiber, of which the following is a specification.

This invention relates to the production of 10 sheets, plates, boards, or other formed or shaped articles comprising a fibrous base impregnated with an agent which preferably at least has cementitious properties, and is capable of acting as a binder for the fiber, 15 or as a waterproofing agent therefor, or is capable of imparting fire-resisting qualities to a combustible fiber. My invention comprises a method of producing such impregnated sheets, articles, or like bodies, and will 20 be described by reference to certain illustrative embodiments thereof, it being understood that the invention is not restricted to the manipulative details hereinafter described, or to any particular proportions of 25 the components, which will necessarily vary widely according to the intended use of the product. The invention is applicable to the production of a great variety of articles, including building-boards, sheets or plates, 30 roofing materials, aeroplane wings, various hollow articles, including bottles, drums, and other containers, etc. An illustrative embodiment of my invention is as follows:—

A suitable fibrous material, for example 35 wood pulp, sulfite fiber, other vegetable fiber, or fibrous asbestos, is beaten up and suspended in water and then deposited upon a suitable foraminous support, for example a metallic cloth or screen, the meshes of which 40 are sufficiently small to retain the fiber; or other fabric or porous body may be used. Suction is applied beneath this support in such manner and in such degree that the fiber is deposited upon the support in a highly 45 compact and closely interlaced condition, the liquid draining through the support. In this way any desired thickness of fibrous sheet or body may be built up. The foraminous support may have any desired form 50 or contour according to the shape of the article to be produced, consisting for example of a flat or curved sheet, a hollow form or the like. In the latter case the fiber may be deposited either upon the outside or upon

the inside of the form, the suction being of 55 course applied to the opposite side of the support.

The impregnation of the fibrous body thus formed is carried out without removing it from the foraminous support, and either 60 with or without preliminary drying, according to the nature of the impregnating solution. If the latter is an aqueous solution, preliminary drying will not as a rule be necessary; whereas drying is desirable or 65 necessary when non-aqueous varnishes or solutions are used for impregnation. In any case the impregnation is preferably carried out while the fiber layer is still held by the suction against its foraminous support, 70 since thereby any pulping or loss of compactness of the fiber is prevented, while on the other hand, an extremely rapid, thorough and intimate impregnation is secured. The impregnating liquid or solution is caused to flow through the body of the 75 fibrous sheet or article until a complete and uniform impregnation is secured.

When the principal effect sought is to 80 fireproof cellulose fiber, any of the known fireproofing salts or agents may be used, including magnesium chlorid, soluble phosphates and the like. Similarly, any suitable waterproofing composition, including asphaltic, resinous or other varnishes, rubber 85 solutions, etc., may be used.

A highly advantageous embodiment of the invention is carried into effect as follows: The fiber, either before being suspended in water or after being so suspended and before 90 being deposited upon the foraminous support, is intimately mixed with a small proportion, say 1-15 per cent., more or less, of calcined magnesia. Suction is then applied to the opposite side of the support, and the 95 mixture of fiber and magnesia is deposited thereon in the form of a highly compact bed or layer. A magnesium chlorid solution, for example the bittern water which is the usual by-product of seaside salt works is 100 then drawn through this bed, whereby the magnesia contained therein is converted into the highly cementitious oxychlorid, the bed being in the meantime strongly compacted, under the suction. In this operation, as in 105 those before described, it is desirable to employ as high a degree of vacuum as is practically attainable, since the higher the

vacuum the more compact the deposit will be. The suction may be maintained until the oxychlorid cement has set sufficiently to prevent any material loosening of the bed or loss of compactness when the pressure upon the two sides is equalized.

While I prefer in all cases to bring about the deposition of the fibrous bed or layer and its impregnation through the influence 5 of suction applied to the opposite side of the foraminous support, my invention contemplates also the establishment of a pressure difference upon opposite sides of the sheet or article to be impregnated by any means, including the application of excess or super-atmospheric pressure to the side of the support upon which the fiber has been deposited.

It is easily possible by this method to produce in a single operation sheets or plates 10 containing an interior reinforcing member, as for example a wire mesh or the like. For this purpose it is only necessary to put the reinforcing member in its proper position upon the foraminous bed, and then to apply 15 the fiber as before until the reinforcing member is properly embedded. Thereafter the impregnation of the fiber layer may be carried on as before. In this way, extremely 20 light, strong and durable structures may be prepared, adapted for any of the purposes 25 heretofore mentioned.

The accompanying drawing illustrates a simple form of apparatus suitable for carrying out the method, the figure being a vertical sectional view. In this figure, 1 illustrates a suitable support or container connected with a suction device by one or more pipes 2. 3 indicates the foraminous bed supported in any suitable manner within 30 the container 1. The article 4 being molded is here indicated as a flat plate or board, but obviously may be of any desired form, depending upon the contour of the foraminated bed. An embedded reinforcing ele-

ment such as a wire mesh, is indicated at 5, 45 which, however, may be omitted.

I claim:—

1. Method of producing an article comprising a fibrous body and a cementitious binder, which consists in forming the article upon a foraminous support from a mixture containing fiber and magnesia, and then subjecting the formed article while carried by said support to the action of a solution of a magnesium salt. 50

2. Method of producing a sheet or article comprising a fibrous body and a cementitious binder, which consists in depositing a mixture of fiber and magnesia upon a foraminous base to form the article, and then treating the formed article while carried by said support with a solution of a magnesium salt while maintaining a difference of pressure 60 on opposite sides thereof.

3. Method of producing an article comprising a fibrous body and a cementitious binder, which consists in suspending a fiber and magnesia in a liquid, depositing them simultaneously therefrom in the form of a sheet or article upon a foraminous support, 70 and then treating the deposited layer while carried by said support with a solution containing magnesium chlorid to convert the magnesia into oxychlorid. 75

4. Method of producing an article comprising a fibrous body and a cementitious binder, which consists in suspending a fiber and magnesia in a liquid, depositing them simultaneously therefrom in the form of a sheet or article upon a foraminous support, 80 and then causing a solution containing magnesium chlorid to flow through the deposited layer while carried by said support until the magnesia therein is converted into oxychlorid. 85

In testimony whereof I affix my signature.

DAVID C. COLLIER.